

Feb. 21, 1961

J. M. FLACK ET AL  
TREATMENT OF FIBERS

2,972,220

Filed Aug. 4, 1955

2 Sheets-Sheet 1



INVENTORS.  
JAMES M. FLACK  
BENJAMIN F. PULSIFER  
JAMES D. WHATLEY

Feb. 21, 1961

J. M. FLACK ET AL  
TREATMENT OF FIBERS

**2,972,220**

Filed Aug. 4, 1955

2 Sheets-Sheet 2



## 1

2,972,220

## TREATMENT OF FIBERS

James M. Flack, Westford, Mass., Benjamin F. Pulsifer, Nashua, N.H., and James D. Whatley, Cordova, Ala., assignors to Indian Head Mills, Inc., New York, N.Y., a corporation of Massachusetts

Filed Aug. 4, 1955, Ser. No. 526,508

7 Claims. (Cl. 57—156)

This invention relates to a novel method of treating cotton in loose fiber form to improve its weaving and spinning properties and to the product which is thereby obtained. The invention relates, in particular, to a method for improving the quality or grade of cotton and for reducing loss in the form of lint waste that normally occurs in the processing of cotton fibers.

In the preparation of cotton thread from the staple, cotton fibers from the bale are subjected to an opening operation followed by cleaning, lint removal, picking, carding, drawing and spinning. One or more of such processing steps has usually involved the separation of short and immature fibers which have heretofore been considered to be undesirable in a high quality cotton thread because it had been found that, unless the short and immature fibers were removed, the spinning of the fibers would be impeded and the resulting product would be weak and of inferior quality. On the other hand, raw staple which had a low content of such short or immature fibers and which would therefore be subject to less loss during processing would be less plentiful and of high cost.

The invention described herein provides a method for treating cotton in loose fiber form so that the short and immature fibers need not be removed but remain in the material thereby effecting an economy in the price and quantity of the staple that may be used without impeding the spinning of the fibers and without loss of quality in the finished product. Another advantage of the invention is that the resulting product has a quality as evidenced by tensile strength and Micronaire count substantially better than it would otherwise have. The short and immature fibers are so modified according to the process of the invention that cotton containing such fibers may be successfully spun into thread of desirable properties.

Particular advantages of the invention are that the amount of lint waste normally lost in processing untreated cotton is greatly reduced; spinning characteristics of the fiber are improved; Micronaire count is substantially increased; and tensile strength is increased.

According to the method of the invention, loose cotton fibers are treated with a cold, strong causticizing agent to swell the fibers without producing substantial gelatinization thereof, while holding the fibers under tension and surface frictional restraint to retard the normal contraction and curling thereof that would occur but for the tension. The tension is applied until the causticizing agent is removed from the fibers. The fibers treated by the method described herein have improved properties from the standpoint of maturity (measured by standard Micronaire tests) and spinability into yarns or threads. Fiber loss in the form of lint waste is lower. The improved properties are thought to be due to the fact that the immature fibers are swollen thereby improving maturity as measured by the Micronaire count.

The cotton subjected to causticizing treatment according to the invention may be wetted raw unscoured cotton; or scoured and wetted; or scoured, bleached and wetted.

## 2

If desired, the causticizing treatment may be carried out on dry fibers. However, it is preferred to moisten the fibers prior to causticizing treatment. More marked and rapid effects are produced by treating scoured, bleached and wetted fibers.

- 5 The length of the fibers is in the textile fiber range, that is, a major portion of the fibers are of length of at least one-half inch, preferably at least  $\frac{3}{4}$  of an inch and ranging up to  $1\frac{1}{2}$  inches or greater length.
- 10 Prior to the causticizing or wetting and causticizing treatment, the fibers may be processed according to usual procedures. The raw cotton fibers are taken from the bale and processed through an opening and cleaning line that will open and fluff up the fibers, clean out non-lint waste without removing immature fibers, and form a mat suitable for chemical treatment. Any suitable means may be employed for initially assembling the fibers. For instance, fibers from the bale after opening, cleaning and lap forming are preferably subjected to a parallelizing treatment, as described in more detail hereinafter, and then the causticizing or wetting plus causticizing process. The weight of the web or lap of dry assembled fibers subjected to causticization is preferably 4 to about 10 ounces for a one yard long section of 40 inch wide web.
- 15 20 25 The web in the weight range indicated is sufficiently light so as not to interfere with the operation of the means described more fully hereinafter which tends to maintain the fibers under tension by frictional restraint during the treatment with causticizing agent. On the other hand, the web is not so heavy that the innermost fibers do not become sufficiently wetted nor sufficiently subjected to the causticizing agent. The preferred maximum web weight is about 14 ounces.
- 30 35 The temperature and time of treatment and concentration of caustic are interrelated and controlled at levels which will produce the desired swelling and controlled curling of the fibers without producing substantial gelatinization thereof. Excessive gelatinization would result in an undesirable welding or fusion of fibers to each other. Generally, the concentration of caustic should be at least 8% and less than 32% NaOH and the temperatures should be from just above the freezing point of the solution to  $85^{\circ}$  F. Preferably, such solutions are used in concentration in the range 20-25% at temperatures of  $14-20^{\circ}$  F. The time of contact between the fibers and the causticizing agent is such as to wet the fibers thoroughly and permit the desired swelling thereof. The time of treatment may be within the range of about 30 seconds to 2 minutes, and, preferably, within the range of 30 seconds to 1 minute.
- 40 45 50 The means and the methods for retaining the fibers under frictional restraint to produce the controlled tension which is an essential element of the invention will be described in greater detail in connection with the graphical description of the invention appearing in the attached Figures 1 and 2.
- 55 Figure 1 is a flow sheet outlining the operating steps, including those which precede and those which follow the causticizing treatment;
- 60 Figure 2 is an illustration, largely schematic, of apparatus for carrying out the method of the invention.
- 65 70 In Figure 1, reference number 10 designates an opening apparatus which loosens the fibers as they come from the bale. After opening, the fibers pass to a cleaner 11 which serves to separate from the cotton foreign material other than lint. Suitable cleaners are the gin cleaner or superjet cleaner with a condenser.
- 75 After opening and cleaning, the fibers pass to the blending reserve, evener and picker, designated generally at 12. The apparatus is operated according to conventional procedure except that the grids of the picker are closed so as to retain substantially all of the shorter fibers. The

picker lap may be introduced directly to the chemical treatment operation illustrated more fully in Figure 2, or may receive an optional but preferably supplemental treatment, for parallelization of the fibers, as shown at 15, prior to the causticizing step. Parallelizing of the fibers may be effected by carding or garneting plus drawing or similar methods which will place the fibers in the form of a sheet or web at least partly but not necessarily completely oriented in one direction, most suitably in the direction of the length of the web.

After the chemical treatment described more fully below, the fibers are dried, suitably in a circulated hot air oven or by infrared radiation, as shown at 17, and opened again at 18 to disperse the fibers suitably in a gin type opener. The opened fibers pass through a blending reserve, evener and picker with the grids closed, as shown at 20, and then through conventional equipment such as carding, drawing, spinning and weaving machines at 21.

Referring to Figure 2 for the details of the wetting and causticizing treatments, reference number 25 designates a roll of specially prepared cotton lap. The lap 26 is unwound from roll 25 by being drawn continuously between the feed rolls 27. Screen belts 30 and 31 above and below the lap, respectively, pick up the lap 26. Screen belt 30 is fed over a series of rollers shown in the drawing above the lap, and screen belt 31 is fed from a series of rollers, some of which are in wetting tank 32 disposed below the lap. Screen belts 30 and 31 converge and come into direct contact with the top and bottom surfaces of the lap so as to carry it down into wetting out solution 35 maintained in tank 32. Belts 30, 31 carry the fibers down into solution 35 and around guide rolls 36 which allow the fibers to remain in the liquid until the fibers are thoroughly wetted.

The fiber lap leaves the screen belts 30, 31 at guide rolls 40 and is fed between squeeze rolls 41. Rolls 41 are driven by suitable means, not shown, as are feed rolls 27 and guide rolls 36 so that the surface speed of screens 30 and 31 will be the same as the surface speed of squeeze rolls 41. If desired, however, the surface speed of screens 30 and 31, as controlled by the cooperating guide rolls, may be varied in relation to the surface speed of squeeze rolls 41.

After leaving squeeze rolls 41, the fibers are again picked up by a pair of screen belts 42 and 45 carried and driven by a series of guide rolls 46 and 47, respectively. Screen belts 42, 45 carry the fibers down into causticizing solution 50 in the tank 51. The lower screen belt 45 passes around weighted guide roll 72 which keeps the screen tight. The top screen belt 42 passes around weighted guide roll 71 which keeps this screen tight and the fiber lap 26 under desired controlled compression between the two screens. The composite screen-fiber web-screen laminate passes around synchronized rollers 55 within the tank.

An important feature of the invention referred to hereinabove is that screens 42 and 45 compress the lap 26 so that the individual fibers are retained in frictional restraint largely through fiber to fiber contact between the wires of the screen mesh and thereby retained under controlled tension to prevent unrestrained shrinkage and curling. The desired conditions of frictional restraint and tension are maintained while the laminate passes through solution 50 in tank 51. Solution 50 is maintained at the desired temperature by a refrigeration apparatus shown in the drawing below tank 51. Solution 50 overflows dam 56 and is withdrawn through piping 57 to pump 60. In the cooler 61, the temperature of the solution is reduced by indirect heat interchange with refrigerant entering the cooler at 62 and leaving at 65, and is then returned to tank 51 through piping 66.

The length of tank 51 and number of cylinders 55 within the tank and the rate of travel of the screens and web through the tank are sufficient to provide the desired

time of contact between causticizing agent 50 and web 26 at the temperature of solution 50.

The endless screen belts 42 and 45 are separated at guide rolls 67 and the separated web is fed between squeeze rolls 70 which squeeze out the excess caustic liquid and return it to tank 51.

After the fiber lap leaves squeeze rolls 70, it is again picked up by a pair of endless screen belts 75 and 76 which carry the cotton lap 26, still under compression, 10 through the first wash box 77. In this box there is a continuous flow of water at about 100° F. through manifolds and jets 80 which impinge directly on the screens and fibers to wash out caustic therefrom. Wash tank 77, and all of the succeeding tanks, have a continuous inflow 15 and outflow of liquid and a liquid level maintained therein by means not shown. After the first wash, the lap leaves the screen belts at rolls 81 and is immediately picked up by squeeze rolls 82 and fed again between a pair of continuous screen belts 85 and 86 and passed 20 through the second washing tank 87. The web leaves belts 85 and 86 at 90 and is passed between the squeeze rolls 91. It is again picked up by screen belts 92 and 95 and passed through tank 96 where it is treated with a diluted solution of acetic acid, sulphuric acid or sodium bicarbonate to neutralize any caustic which still remains 25 in the fibers.

The fiber lap 26 is then carried through squeeze rolls 100 and thence through wash tanks 101 and 102 between endless cooperating screen belts in each case and through 30 a squeeze roll after each wash. In each tank there is a substantial flow of hot water through piping, not shown in the drawing, for the purpose of washing out residual amounts of chemicals which may remain in the fibers. Finally, the cotton lap 26 reaches tank 105 where it is again treated with a liquid between parallel cooperating 35 endless belt screens. The liquid in tank 105 is a solution or an emulsion 106 of a fiber lubricant. It is finally squeezed between rolls 107 and passes along to a raw stock dryer, not shown in the drawing.

The mesh of the screen is of some importance in obtaining successful results according to the invention. The screen mesh generally must be sufficiently open to permit passage of the causticizing liquid and thorough wetting and treatment of all the fibers. On the other hand, it 40 must be sufficiently fine to retain the fibers under frictional restraint and controlled tension so as to retard and control the extent of shrinkage of the fibers during causticizing. The mesh also must be sufficiently fine to prevent excessive loss of small fibers through the screen. Screens having four meshes to the inch have been used 45 successfully according to the method of the invention. Generally, the screen opening may be about  $\frac{1}{16}$  inch to as much as about  $\frac{1}{4}$  inch without resulting in appreciable loss of the shorter fibers and without sacrificing desired 50 frictional restraint of the fibers during causticization.

Following is an example of one mode of carrying out the process of the invention and of manufacturing the product of the invention.

#### Example

60 A 14 ounce picker lap of loose cotton fibers, which had been opened from the bale, cleaned and processed through the picker, was placed between two  $\frac{1}{4}$  inch mesh screens, pressed together and treated in the following manner:

65 (1) Immersed in a cold aqueous solution of two pounds of "Kwik Wet" wetting agent (produced by Edwal Scientific Products Company) per 50 gallons of water for 10 seconds. The excess water was then squeezed out by running the screens and the web through rubber covered 70 squeeze rolls under pressure. Other wetting agents may be substituted for the "Kwik Wet."

(2) Immersed in an aqueous sodium hydroxide solution (50 gallons) 48° Twaddell at 20° F. The caustic solution contained 4 pounds, 6 ounces of "Dypenol No. 75 88" wetting agent (produced by Dexter Chemical Corp.).

The initial immersion period was 5 seconds after which the screens and web were passed between rubber covered squeeze rolls under pressure to squeeze out excess caustic. About ten seconds after removing the web from the caustic bath in the first immersion period, the web was submerged for a second immersion period in the same caustic and held there for 35 seconds. After the second immersion period, excess caustic was squeezed out between rolls as before. The total time of contact of the fibers with caustic was 50 seconds. Other types of wetting agents suitable for use as aqueous solutions may be substituted for the "Dypenol No. 88."

(3) Washed in running water at 160° F. for ten seconds and thereafter again squeezed between rolls under pressure.

(4) Washed in running water at 160° F. for ten seconds and compressed as before.

(5) Immersed in an aqueous solution of 5 pounds sodium bicarbonate per 50 gallons of water at a temperature near boiling for 10 seconds and thereafter compressed between rolls under pressure to remove excess solution. Sodium bicarbonate may be replaced by acetic acid or sulphuric acid (dilute in each case) for the same purpose, i.e., the removal of residual amounts of sodium hydroxide which may be retained by the fibers.

(6) Washed in running water at 160° F. until all alkali was removed from the fiber. At the end of this washing period, the pH of the fibers was 7.0 to 7.2.

(7) Immersed in an aqueous solution or emulsion of a fiber lubricant of a type known in the textile fiber field. The amount of lubricant deposit on the fiber is not over 0.2 part of 1% based on the weight of the dry fiber. After immersion, the excess lubricant is removed by squeezing as before.

(8) The screens are removed from the fiber web and the fibers passed through a hot air type drier to dry the fibers.

(9) The caustic treated and dried fibers are processed in conventional gin type opener and picker followed by usual mill processes, i.e., carding, drawing and spinning. The fineness of the treated fiber, as determined by Micronaire measurement, was 3.8 as compared with a value of 2.5 determined by measurement of the fineness of untreated fiber. This reflects an increase in coarseness of the fiber of about 50% since the higher reading on the Micronaire reflects a lower degree of fineness.

Although specific embodiments of the invention have been described herein, it will be apparent to those skilled in the art that the invention contemplates many modifications and equivalents. Accordingly, it is intended to include within the scope of the appended claims all modifications and equivalents of the invention.

We claim:

1. The method of treating loose unwoven cotton fibers containing immature fibers which comprises compressing a web of said fibers between parallel screens to provide surface frictional restraint to prevent normal shrinkage and curling of said fibers during treatment with caustic cellulose swelling agent, treating said web while it is compressed between said screens with a strong caustic cellulose swelling agent of sufficient strength to produce chemical swelling thereof at such temperature and for such duration as to swell said fibers without substantial gelatinization thereof, the strength of said agent being sufficient under said conditions of temperature and duration of treatment to produce shrinkage and curling of said fibers in the absence of said frictional restraint, thereby to increase the measured maturity of the finished fiber web, removing the caustic

cellulose swelling agent from said fibers while said fibers are still held by surface frictional restraint, removing said fibers from said screens thereby to obtain a web which can be processed into a thread, orienting the treated fibers in said web for spinning and spinning said oriented fibers into a thread.

2. The method of claim 1 in which the dry weight of the fiber web is in the range of approximately 4 to 14 ounces for a one yard length of 40 inch wide web.

10 3. The method according to claim 1 in which the cellulose swelling agent is an aqueous NaOH solution of concentration in the range of approximately 8-32% and temperature in the range from but not including the freezing point of the solution to approximately 15 85° F.

4. The method of claim 1 in which the fibers are pre-wetted with water before they are treated with cellulose swelling agent.

20 5. A thread prepared by spinning fibers produced by the method of claim 1.

6. In the method of preparing a cotton web suitable for drawing and spinning into a thread comprising the steps of opening, cleaning, picking and carding the fibers, the improvement which comprises retaining in the fiber mass 25 the short and the immature fibers normally removed before spinning, compressing said fibers at a stage in the operation subsequent to the cleaning stage in the form of a web between parallel screens to provide surface frictional restraint to prevent normal shrinkage and curling of said fibers during treatment with caustic cellulose swelling agent, treating said compressed web with a strong caustic cellulose swelling agent of sufficient strength to produce chemical swelling thereof at such temperature and for such duration as to swell said fibers

30 without substantial gelatinization thereof, the strength of said agent being sufficient under said conditions of temperature and duration of treatment to produce shrinkage and curling of said fibers in the absence of said frictional restraint, thereby to increase the measured maturity 35 of the finished fiber web, removing said caustic cellulose swelling agent from said fibers while said fibers are still compressed between said screens, removing said fibers from said screens thereby to obtain a web which may be processed into a thread of satisfactory quality 40 containing said short and said immature fibers, orienting the treated fibers in said web for spinning, and spinning said oriented fibers into a thread.

45 7. The method described in claim 1 wherein the fineness of said loose unwoven cotton fibers containing immature fibers as measured by Micronaire count is about 2.5.

#### References Cited in the file of this patent

#### UNITED STATES PATENTS

|           |          |       |              |
|-----------|----------|-------|--------------|
| 1,626,766 | Tompkins | ----- | May 3, 1927  |
| 1,757,755 | Hahn     | ----- | May 6, 1930  |
| 1,757,756 | Schwartz | ----- | May 6, 1930  |
| 1,757,757 | Schwartz | ----- | May 6, 1930  |
| 1,791,248 | Schwartz | ----- | Feb. 3, 1931 |
| 2,528,793 | Sechrist | ----- | Nov. 7, 1950 |
| 2,552,078 | Williams | ----- | May 8, 1951  |

#### FOREIGN PATENTS

|           |               |       |              |
|-----------|---------------|-------|--------------|
| 65 17,397 | Great Britain | ----- | A.D. 1897    |
| 443,888   | Great Britain | ----- | Dec. 8, 1934 |

#### OTHER REFERENCES

Textile Research Journal, February 1954, pp. 156-70 172.

UNITED STATES PATENT OFFICE  
CERTIFICATION OF CORRECTION

Patent No. 2,972,220

February 21, 1961

James M. Flack et al.

It is hereby certified that error appears in the above numbered patent requiring correction and that the said Letters Patent should read as corrected below.

Column 6, list of references cited, under "UNITED STATES PATENTS", add the following:

2,774,126 Secrist ----- Dec. 18, 1956

Signed and sealed this 11th day of July 1961.

(SEAL)  
Attest:

ERNEST W. SWIDER  
Attesting Officer

DAVID L. LADD  
Commissioner of Patents